

March 4, 1924.

1,486,015

C. B. FILBERT

ROAD AND METHOD OF WATERPROOFING THE SAME

Filed Oct. 14, 1922



INVENTOR.  
*Calvert Burke Filbert*  
BY  
*William O'Reane*  
his ATTORNEY

Patented Mar. 4, 1924.

1,486,015

# UNITED STATES PATENT OFFICE.

CALVERT BURKE FILBERT, OF NEW ORLEANS, LOUISIANA.

## ROAD AND METHOD OF WATERPROOFING THE SAME.

Application filed October 14, 1922. Serial No. 594,588.

*To all whom it may concern:*

Be it known that I, CALVERT BURKE FILBERT, citizen of the United States, residing at New Orleans, in the parish of Orleans and 5 State of Louisiana, have invented certain new and useful Improvements in Roads and Methods of Waterproofing the Same, of which the following is a specification.

In the ordinary methods of oiling or 10 waterproofing macadam, gravel, shell, slag, chert roads and the like, the surface of the roadway is generally swept free of loose material and a single application of bituminous material is applied to the roadway and 15 coated with chips, shells, sand or other suitable mineral aggregate. In many instances, however, the oil or other bituminous material is thin or light in body and is completely absorbed by the road surface. Consequently 20 the oil fails to provide the necessary adherence of the surface dressing of chips, etc., heretofore mentioned. In other cases, where the oil is sufficiently heavy to insure the necessary adherence of the surface 25 dressing of chips and the like, there is frequently little or no penetration into the road structure, that is, the road itself does not absorb the oil, and consequently the surface coat of oil and mineral aggregate is subject 30 to pushing and waving from traffic and often completely separates itself from the road structure.

The primary object of the present invention is to eliminate the disadvantages in the 35 known methods and to improve the roads treated by my process. In practicing my invention, the oils or other water-proofing mediums are applied to the road surface in two or more successive stages using two different 40 grades or qualities of material, the first of these materials being capable of insuring penetration into the road structure, while the second provides a firm bond or union with the first and with the carpet coat of mineral aggregate which serves as a wearing surface.

The drawing forming a part of this application shows a cross-section of the road constructed in accordance with the method disclosed, and bearing the legend reciting the steps of the method.

In the first stage or application of the invention, I employ an oil containing preferably from 45 to 65 per cent asphalt and of 55 relatively thin fluidity, so that it may if desired be applied to the road surface in a cold

state, or the oil may be slightly heated, if necessary. The asphalt content, temperature, and extent of application of the oil will depend on the texture and density of the old road surface. Oils suitable for the primary or priming treatments are preferably relatively high in volatile constituents, so that they should show a loss from evaporation of approximately 15 to 30 per cent by weight when tested by the standard method of the American Society for Testing Materials.

Prior to the application of these priming oils, the dry road surface should preferably be brushed free of loosely bonded material, and as many gravel and chert roads do not have sufficient stability to withstand heavy brushing, such roads should only be slightly swept. After the application of the priming oil by mechanical distribution and usually at the rate of from  $\frac{1}{4}$  to  $\frac{1}{2}$  gallon for one square yard, the surface is left undisturbed and preferably free from traffic a sufficient time to permit the oil to be completely absorbed by the road. In the case of very porous roads, especially the newly constructed water-bound macadams and gravel types, it may be advisable to repeat the treatment with the primary oil, but with a less quantity of the latter. Also any "fat" spots that may remain on account of inequality of density or compaction of the old road structure should be covered with just sufficient dry sand to absorb the excess bitumen, and the sand so added removed prior to the application of the secondary oil.

Volatilization of the lighter constituents of the priming oil after it has been applied to the old road structure results in a "curling" of the road surface due to a hardening or thickening of the oiling material, and the hardening or thickening is progressive in character from the lower layers of the road structure toward the surface or crust.

In the secondary treatment, I preferably use an oil of from 65 to 100 per cent asphalt content, and which is relatively low in volatility that is, materials showing less than 15 per cent evaporation loss by the standard test of the American Society for Testing Materials. These oils are applied to the primed road surface already referred to in a heated condition, and preferably by the use of mechanical distributors. The temperature of application should preferably be between 275 degrees and 375 de-

degrees Fahrenheit and the quantity usually  $\frac{1}{2}$  to  $\frac{1}{4}$  gallon per square yard of road surface, this depending on the texture and density of the old road structure and also 5 on the size of the particles of the material subsequently to be applied as a surface dressing.

After the secondary oil has been applied, and distributed uniformly by squeegees if 10 necessary, the surface dressing of crushed stone chips, gravel, slag, shells, or coarse sand or the like is scattered over the oiled surface in the usual manner and then the road is thoroughly rolled. The usual 15 precautions should be taken to insure that the stone chips, gravel or the like are dry and free from dust and fine material.

By means of this double treatment, the heavy oil used in the secondary application 20 follows the path of the priming oil, and, as it penetrates into the road structures and cools, it attaches itself to the stone, gravel, slag or other road structure that has preferably been oiled by the priming application. A 25 progressive thickening of the bituminous or oiling material occurs as the surface is reached, and at the same time the film of oil remaining unabsorbed is sufficiently tenacious to hold the stone chips or the like 30 added as the surface dressing or new wearing surface.

The present invention provides a road structure in which the surface coat will remain firmly in position for a long time.

From the foregoing, it is believed that the steps of the process and the structure 35 of the road formed thereby may be readily understood by those skilled in the art and it is apparent that various changes may be 40 made in the details disclosed without departing from the spirit of the invention as expressed in the claims.

What is claimed and desired to be secured by Letters Patent is:

1. A method of treating ready made road structures having a surface portion of 45 porous mineral aggregate, consisting in first removing dust from the surface portion, then applying a priming water-proofing 50 liquid containing asphalt to the remaining rigid road surface, allowing the major portion of said liquid to be absorbed by the road structure, applying to the road a heavier liquid water-proofing material containing asphalt in a greater proportion than 55 said priming liquid, and then adding a surface dressing of mineral aggregate substantially coarser than common road dust, upon the second water-proofing material.

2. A method of treating an old road structure having a surface portion of porous

mineral aggregate, consisting in first applying to the surface of a road structure a priming water-proofing liquid medium containing asphalt and capable of penetrating 65 into and binding the elements of the road structure, then applying at a temperature at which it is liquid, a second water-proofing medium containing asphalt, in a greater proportion than does said priming liquid, 70 and capable of bonding with the first water-proofing medium and providing surface adherence, and finally applying a surface dressing of mineral aggregate upon the second water-proofing medium. 75

3. A method of treating road structures consisting in first removing dust from the surface of the road structure, then applying to the surface of the road structure a relatively thin asphalt-containing oil capable of penetrating the road structure and also capable of partial evaporation at atmospheric temperature, then applying a less volatile asphalt-containing water-proofing medium, at a temperature at which it is 80 liquid, capable of bonding with said oil and providing surface adherence, and then adding a surface dressing of mineral aggregate upon said road, and compacting the surface. 85

4. A method of water-proofing macadam, gravel, slag, shell, chert roads or the like consisting in applying a relatively thin volatile asphaltic oil to the road surface and after the major portion of said oil has been 90 absorbed by the road and a minor portion of the same has been evaporated applying in a liquid condition, a water-proofing medium of heavier less volatile asphaltic oil capable of bonding to the first mentioned oil 95 and the road surface. 100

5. In the treatment of old roads, the herein described improvement which comprises applying to a porous hard old road surface, which is substantially free from top dust, 105 a priming coat of a thin liquid asphaltic oil, and allowing the major portion thereof to permeate into the hard road body; thereafter applying to such road surface, a viscous asphaltic material in a freely liquid 110 state, such latter material containing a substantially higher percentage of asphalt than the oil used in said priming coat, spreading out said second applied liquid asphaltic material, then applying hard granular road metal of a size much coarser 115 than ordinary road dust upon said second applied asphaltic material, and finally rolling said structure.

In testimony whereof I affix my signature.

CALVERT BURKE FILBERT.